

Patented Feb. 23, 1926.

1,574,375

# UNITED STATES PATENT OFFICE.

WILLIAM J. DIEDERICHS AND ANSON HAYES, OF AMES, IOWA.

## PROCESS FOR TREATING IRON.

No Drawing. Original application filed August 21, 1922, Serial No. 583,370. Divided and this application filed August 6, 1925. Serial No. 48,623.

To all whom it may concern:

Be it known that we, WILLIAM J. DIEDERICHS and ANSON HAYES, each a citizen of the United States of America, and resident of Ames, Story County, Iowa, have invented a new and useful Process for Treating Iron, of which the following is a specification.

The subject matter of this application was originally included in but has been divided 10 from our application filed August 21, 1922, Serial Number 583,370.

The object of this invention is to provide a new and improved process for treating white cast iron whereby an iron is produced 15 practically duplicating the properties of commercial malleable iron, and in a much shorter time than now required in the ordinary malleabilizing process.

A further object of this invention is to 20 shorten the time required for producing malleable iron.

These and other objects of the invention will be more clearly described in the specification and pointed out in the appended 25 claims.

Any suitable type or form of furnace or so-called annealing oven may be employed in carrying out our improved process, and may be heated by any of the well known 30 forms of fuel such as gas, oil, or powdered coal burned in connection with air; or the heat may be secured electrically or by a combination of combustion and electricity, or in any other manner that may be desired 35 so long as the desired temperatures and atmospheres are attained.

The iron used in this process is known as white cast iron such as is used in making malleable castings. This white cast iron 40 differs principally from ordinary gray iron in that while both contain carbon the white cast iron contains the carbon wholly or principally in the form of carbide of iron represented by the formula  $Fe_3C$ , while 45 gray cast iron contains the carbon to a greater degree in the form of graphite or graphitic carbon.

It is well known that ordinarily in making malleable castings the white iron is 50 packed with some packing material in sealed boxes or pots which are loaded into the furnace while the furnace is cold and the furnace is then gradually raised to a temperature of between 800 and 850 degrees centigrade and maintained at that tempera-

ture for approximately sixty hours, after which the furnace is gradually cooled, the whole process requiring seven to nine days of continuous operation. In the making of malleable castings the iron carbide is 60 changed mainly to iron and temper carbon or graphite, the resulting iron usually having a lower tensile strength than the white cast iron from which it was made, but it will bend or stretch to an appreciable degree, which is not true of the white cast iron.

In carrying out our improved process we use the white cast iron just as in the process above described, but we employ a very different and much shorter process, which may involve higher temperatures at times. By this process we obtain a product fully as characteristic and practically duplicating all 75 the properties of malleable iron produced by the now common and well known methods, but in a much shorter time.

In carrying out this process we do not necessarily pack the white iron castings as 80 in the ordinary malleabilizing process, although that may be done at times if desired. By omitting it considerable time is saved. When the packing is omitted the white iron castings may be supported in any suitable manner in the furnace to prevent sagging and warping under the intense heat. The process consists in heating for any length of time, raising the temperature of the white iron castings with convenient rapidity, 85 either rapidly or slowly, to any point between critical temperature of the material (about 740 degrees centigrade) and the point of incipient fusion, and holding at the chosen higher temperature for a period of fifteen minutes to five hours, or more. The

actual time required will depend upon the temperature chosen, lower temperatures requiring longer times, and upon the chemical composition of the white iron being treated. In any case it is only desired to maintain the higher temperature until the massive cementite is practically all absorbed in the solid solution. We are satisfied that in most instances it would avail little to hold at the high temperature for a longer period than about five hours, since practically all of the desirable change would have occurred in that time, especially if the high temperature employed is above 900 degrees centigrade; and that holding for longer periods 100

105

110

would result only in waste of time without corresponding benefit. If a high temperature of less than about 900 degrees centigrade is used the time required to practically complete the absorption of massive cementite into the solid solution will be very materially increased.

The castings may then be removed from the furnace and cooled by quenching in any suitable material such as sand, cement, powdered mica or the like; or they may be cooled in any suitable manner. These operations may be repeated for any desired number of repetitions, that is to say, the material may be alternately heated to a point above the critical temperature and then cooled rapidly to a temperature considerably below the critical. The number of repetitions or alternate heating and coolings, as well as the rates of heating, may be varied in accordance with the properties desired in the product.

The final step of the process consists in making the final cooling extremely slowly, preferably at the rate of about five degrees centigrade per hour. This is the step which insures and characterizes the product as malleable iron, as by the addition of this step a product is obtained duplicating approximately the characteristics and properties of commercial malleable iron, that is having a tensile strength of from 44,000 to 53,000 pounds per square inch or more, and an elongation or ability to stretch of ten percent or more, in two inches. The process is much shorter than that now carried out to obtain commercial malleable iron, the saving in time depending considerably, of course, upon the number of repetitions of heating and cooling employed in a particular instance.

We have also found that by a combination of the high temperature followed by a repetition of alternate heating and cooling; or vice versa, that is alternate heating and cooling with a higher temperature either following or interposed, and in any event followed by an extremely slow cooling, we obtain a resulting material of the same properties as that obtained by either one of the methods individually.

When speaking of the critical temperature of the material, the fact should be borne in mind, which is well known in metallurgy, that the critical temperature can be, and is, undercooled by a rapid cooling, and therefore will be reduced by heating to a temperature above the critical and cooling fairly rapidly; so that in thereafter heating to the critical temperature, it is obvious that a lower actual temperature will be involved. The language of this specification and the appended claims is used with this fact in mind and should be so construed.

The particular thing which characterizes

our present invention and process, and differentiates from the process disclosed and claimed in our parent application above referred to, is that in the present instance the cooling, after each heating to a point above the critical temperature, is continued until comparatively low temperatures are reached. This may be accomplished, if desired, by removing from the furnace and quenching in some suitable material, which obviously results in further saving of time, but requires more handling of the material.

As an example of our experiments in conducting this process, we heated bars of white cast iron to about 1000 degrees centigrade for two hours, cooled in sand to room temperature, reheated to 800 degrees centigrade for six hours, and then cooled very slowly, at the rate of about five degrees centigrade per hour. The resultant product showed a tensile strength of 48,000 pounds per square inch, with an elongation of fourteen percent in two inches.

Likewise by way of illustration, bars of white cast iron were heated to 850 degrees centigrade and cooled to room temperature by quenching in sand, for various numbers of repetitions, the final cooling being at a slow rate of about four degrees centigrade per hour. Bars so heated thirteen times gave a tensile strength of 50,000 pounds per square inch with fifteen per cent elongation in two inches; and bars so heated seventeen times showed a tensile strength of 49,100 pounds per square inch and an elongation of sixteen percent in two inches.

This indicates that a product having the characteristics of commercial malleable iron may be secured by this process in a much shorter time than by the present process, and that the properties may be varied somewhat by the number of successive heatings and coolings to which the material is subjected, and also by the rates of cooling employed.

We claim as our invention—

1. The process for the heat treatment of castings from white cast iron which consists in (1) subjecting of the casting to a temperature above the critical temperature of the material; (2) cooling the casting to a temperature considerably below the original critical temperature; (3) reheating the casting to a sufficient temperature to allow structural and chemical changes to progress; and (4) cooling the casting at an extremely slow rate of about five degrees centigrade per hour.

2. The process for the heat treatment of castings from white cast iron which consists in (1) subjecting of the casting to a temperature above the critical temperature of the material; (2) cooling the casting to a temperature considerably below the original critical temperature; (3) reheating the casting to a sufficient temperature to allow

- structural and chemical changes to progress; (4) cooling the casting to a point where structural and chemical changes cease; (5) alternate repetition of steps (3) and (4); 5 and (6) a final heating to a point where structural and chemical changes can progress, followed by an extremely slow cooling, at the rate of about five degrees centigrade per hour.
- 10 3. The process for the heat treatment of castings from white cast iron which consists in (1) subjecting of the casting to a temperature considerably above the critical temperature of the material for a period of 15 from fifteen minutes to five hours, or more, until the iron carbid present is practically all absorbed in the solid solution, or in other words until in irons of commercial composition the combined carbon is reduced 20 to substantially nine-tenths of one percent; (2) cooling of the casting by quenching; (3) a final heating to a point above the critical temperature; followed by (4) an extremely slow cooling, at the rate of about 25 five degrees centigrade per hour.
4. The process for the heat treatment of castings from white cast iron which consists in (1) subjecting of the casting to a temperature considerably above the critical 30 temperature of the material for a period of
- from fifteen minutes to five hours, or more, until the iron carbid present is practically all absorbed in the solid solution, or in other words until in irons of commercial composition the combined carbon is reduced 35 to substantially nine-tenths of one per cent; (2) cooling the casting to a point where structural and chemical changes cease; (3) a final heating to a point sufficient to allow structural and chemical changes to progress; 40 followed by (4) an extremely slow cooling, at the rate of about five degrees centigrade per hour.
5. The process for the heat treatment of castings from white cast iron which consists in (1) subjecting of the casting to a temperature considerably above the critical temperature of the material for a period of 45 from fifteen minutes to five hours, or more; (2) cooling the casting by quenching; (3) 50 repetition of the above named steps alternately; and a final step consisting in (4) an extremely slow cooling, at the rate of about five degrees centigrade per hour.

Signed at Des Moines, in the county of Polk and State of Iowa, this 18th day of June, 1925.

WILLIAM J. DIEDERICHS.  
ANSON HAYES.